

## UNITED STATES PATENT OFFICE

2,211,535

## ELECTRODEPOSITION OF NICKEL

Henry Brown, Detroit, Mich., assignor, by mesne assignments, to The Udrylite Corporation, a corporation of Delaware

No Drawing. Application June 13, 1938,  
Serial No. 213,454

10 Claims. (Cl. 204—14)

This invention relates to the electrodeposition of nickel from an acid bath.

The object of this invention is to decrease the grain size and increase the lustre of the nickel deposit.

I have found that this object can be accomplished by the addition of certain organic compounds to the standard nickel sulphate baths. These compounds are classed as arsonic acids.

10 Several compounds of this class are listed in Table I with their optimum concentration in baths prepared from nickel sulphate, nickel chloride and boric acid and containing 75 g./l. Ni, 15 g./l. chloride and 35 g./l. boric acid. The 15 temperature of the plating solution can range from room temperature to boiling and preferably from room temperature to 55° C., ordinarily 50° C. The pH of the solution may vary between 1.5 and 3.5 and preferably 2.0—3.0. The preferred 20 current densities range between 4.0 and 7.5 amp./sq. dm.

The presence of other inorganic salts such as NH<sub>4</sub> and Na salts does not interfere with the beneficial action of these organic compounds as 25 long as inorganic materials are present in such amounts which are common in ordinary white nickel baths. Thus the invention is not limited to any specific nickel plating bath.

| 30                                                                                       | Table I | Grams per liter |
|------------------------------------------------------------------------------------------|---------|-----------------|
| Phenyl arsonic acid, C <sub>6</sub> H <sub>5</sub> .AsO(OH) <sub>2</sub>                 | 1.0     | —2.0            |
| Benzylarsonic acid, C <sub>6</sub> H <sub>5</sub> .CH <sub>2</sub> .AsO(OH) <sub>2</sub> | 1.0     | —2.0            |
| n-Butyl arsonic acid, C <sub>3</sub> H <sub>7</sub> .AsO(OH) <sub>2</sub>                | 1.0     | —2.0            |
| 35 Allyl arsonic acid,<br>CH <sub>2</sub> =CH.CH <sub>2</sub> .AsO(OH) <sub>2</sub>      | —       | .75—1.5         |

Lower concentrations than those given in Table I such as .2 g./l. can be used but the effect is not 40 so pronounced. Higher concentrations should be avoided because of preferential plating out of arsenic at low current density points, causing dark plate in recesses.

For best results the over all current density 45 should always be high, of the order of 4.5—6.5 amp./sq. dm. without agitation at 50° C. and pH=2.3. In agitated solutions higher current densities should be used and lower concentrations should be employed to avoid dark plate in 50 recesses.

I have found that the addition of relatively small amounts of arsonic acids, for example, .5 g./l. phenyl arsonic acid to a nickel bath which also contains a sulphonamide (see my copending 55 application Serial No. 162,696, filed September 7,

1937) for example, 2 g./l. o-toluene sulphonamide, or to a bath containing a suitable substituted phenyl sulphonic acid, for example, 2 g./l. thymol sulphonic acid or 2 g./l. dichlorobenzene sulphonic acid (see my copending application Serial No. 213,456, filed June 13, 1938), or a naphthalene sulphonic acid such as 2 g./l. naphthalene disulphonic acid (see United States Patent No. 905,837 to Broadwell) or an alkyl substituted naphthalene sulphonic acid such as 2 g./l. di-isopropyl 5 naphthalene sulphonic acid (see United States Patent No. 1,818,229 to Lutz and Westbrook), produces a degree of grain refinement and brightness which cannot be obtained with these compounds alone, especially at high current densities. To get the most desirable effect the pH 10 should be kept low, between 2 and 3.

I have also found that the addition of small amounts of auxiliary brighteners which plate out with the nickel such as zinc and cadmium in 15 the form of, for example, chlorides or sulphates, and selenium and tellurium in the form of, for example, their oxides or acids, increase greatly the degree of brightness obtained with the arsonic acids. This combination can be used 20 where high ductility and maximum corrosion resistance are non-important. The optimum concentrations of these auxiliary brighteners are 25 given in Table II.

| 30        | Table II | Grams per liter |
|-----------|----------|-----------------|
| Zinc      | —        | .25             |
| Cadmium   | —        | .4              |
| Selenium  | —        | .15             |
| Tellurium | —        | .15             |
|           |          | 35              |

I claim:

1. The method of electrodepositing nickel which comprises electrolyzing an aqueous acid solution comprising essentially a substance selected from the group consisting of nickel sulphate, nickel chloride, and nickel sulphate and nickel chloride together in the presence of an arsonic acid.

2. The method of electrodepositing nickel which comprises electrolyzing an aqueous acid solution comprising essentially a substance selected from the group consisting of nickel sulphate, nickel chloride, and nickel sulphate and nickel chloride together in the presence of an arsonic acid.

3. The method of electrodepositing nickel which comprises electrolyzing an aqueous acid solution having a pH falling within a range of from 1.5 to 3.5 and comprising essentially nickel

55

sulphate, nickel chloride and boric acid in the presence of an arsonic acid.

4. The method of electrodepositing nickel which comprises electrolyzing an aqueous acid solution comprising essentially nickel sulphate, nickel chloride and boric acid in the presence of an arsonic acid in an amount not exceeding approximately 2 grams per liter.

5. A nickel plating bath comprising an aqueous acid solution comprising essentially a substance selected from the group consisting of nickel sulphate, nickel chloride, and nickel sulphate and nickel chloride together, and an arsonic acid.

6. A nickel plating bath comprising an aqueous acid solution comprising essentially nickel sulphate, nickel chloride and boric acid, and an arsonic acid.

7. A nickel plating bath comprising an aqueous acid solution having a pH falling within a range of from 1.5 to 3.5 and comprising essentially a substance selected from the group consisting of nickel sulphate, nickel chloride, and nickel sul-

phate and nickel chloride together and an arsonic acid.

8. A nickel plating bath comprising an aqueous acid solution comprising essentially nickel sulphate, nickel chloride and boric acid and an arsonic acid in an amount not exceeding approximately 2 grams per liter.

9. The method of electrodepositing nickel which comprises electrolyzing an aqueous acid solution comprising essentially a substance selected from the group consisting of nickel sulphate, nickel chloride, and nickel sulphate and nickel chloride together, an arsonic acid and a small amount of a metal from the group consisting of zinc, cadmium, selenium and tellurium.

10. The method of electrodepositing nickel which comprises electrolyzing an aqueous acid solution comprising essentially nickel sulphates, nickel chloride and boric acid, and phenyl arsonic acid.

HENRY BROWN.

20